# EUROPEAN PATENT APPLICATION

(11) **EP 0 308 095 A1**
(43) Date of publication of application: **22.03.1989**
(21) Application number: 88307880.0
(22) Date of filing: 25.08.1988
(51) Int. Cl.: C10L 5/10

(54) **Coal briquetting process**

(30) Priority: 16.09.1987 GB 8721757
(71) Applicant: Coal Industry (Patents) Limited, London SW1X 7AE (GB)
(72) Inventor: Goleczka, Joseph, Cheltenham Gloucestershire (GB); Taylor, Rodney, Evesham Worcestershire (GB); Kelly, Simon, Cheltenham Gloucestershire (GB); Hale, Stuart, Redmarley Gloucestershire (GB)
(74) Representative: Wood, John Irwin (GB)

(57) **Abstract**

Cold coal briquettes of high crushing strength are made by a process comprising mixing fine coal with a binder comprising 5-15% sugar solution of a concentration of at least 25% by weight and up to 5% of hardening accelerator for the sugar solution selected from iron oxide, calcium carbonate, calcium phosphate and aluminium odixe, each optionally with an acid, and p-toluene sulphonic acid. The mixture is formed into briquettes and the resulting green briquettes are hardened.

## Description

This invention concerns a coal briquetting process, and more especially it concerns a process for "cold" briquetting.

There exist many processes for briquetting fine coals in which the mixture fed to the briquetting press is hot, and various binders which melt at the operating temperature, such as pitch are used. In some cases, the coal itself, because it cakes at the operating temperature, forms or contributes to the binder. There is also interest in "cold" coal briquetting processes which require no heating or only heating to about 100° C before briquetting. A binder must be used, therefore, which is effective at low temperatures, and many binders have been suggested. A problem faced especially by "cold" briquetting processes, is that the binders in the product briquettes may not provide adequate binding of the fine coal at or near the combustion temperature, resulting in partial or complete disintegration of the briquette and the loss of coal through the grate. This is termed "undergrate loss".

Our co-pending UK Patent Application No 87/03410 (Publication No. 2 187 754A) discloses a novel cold coal briquetting process utilising a binder which is a mixture of 5 to 15% molasses and up to 5% of an inorganic hardening agent selected from iron oxide, calcium carbonate, calcium phosphate and aluminium oxide, optionally together with an acid, all percentages being by weight of the mix of fine coal and binder.

We have now discovered that concentrated sugar solutions or their closely related starch derivatives may be used in place of molasses. Use hereinafter of the general description "sugar" is to be understood as including such starches. In certain circumstances, such sugar solutions may be more economic to use than molasses, although molasses remains the preferred binder for technical reasons. It has been found that some briquettes made with sugar solutions exhibit a lower green strength, that is their strength immediately after forming the briquette is lower, than briquettes made with molasses, and hence greater care is required in handling the green briquettes to avoid unnecessary breakage. Using a subsequent hot curing step as disclosed in the earlier application results in a rapid gaining of strength, until the crushing strength approaches that of the cured molasses-bound briquettes.

Accordingly, the present invention provides a cold coal briquetting process which is a modification of that of UK Patent Application No 87/03410 (Publication No.2 187 754A), and comprises mixing fine coal with a binder comprising 5-15% sugar solution of a concentration of at least 25% by weight and up to 5% of hardening accelerator for the sugar solution, selected from iron oxide, calcium carbonate, calcium phosphate and aluminium oxide, each optionally with an acid, and p-toluene sulphonic acid, forming the mixture into briquettes, hardening the resulting green briquettes.

Preferred coals are high rank non-caking coals, especially those having low smoke emissions such as anthracite. Desirably the coal is of a particle size mainly below 3mm, and anthracite duff is especially suitable. The invention is also applicable to coals for power stations or steam raising and to coal blends containing caking coal components and/or treated coals e.g. by mild oxidation or by pyrolysis. The coal may be crushed or be the direct product of coal cutting.

The sugar solution preferably contains 50% or more of solids, by weight. It is believed that most refined or unrefined sugars may be used, and the solution may contain other components provided these do not significantly adversely affect the physical and combustion properties of the resulting briquettes.

The hardening agents ferric oxide, calcium carbonate, calcium phosphate, and aluminium oxide, are readily available at low price in such forms as iron ore, limestone, phosphate rock and bauxite. These may be used alone or together in total amounts of 0.5 to 3%. Phosphoric acid or sulphuric acid may be used in amounts of up to 2% in admixture with any one or more ferric oxide, calcium carbonate and aluminium oxide. We have also discovered that an organic acid, p-toluene sulphonic acid, may be used in place of phosphoric or sulphuric acid, either alone or in admixture with the above accelerators. Routine testing should, of course, be carried out to ensure that any individual coal/binder mix is satisfactory.

The briquetting step of the present invention includes all methods of forming agglomerates from fine coal, and these agglomerates may be of any size or shape according to market requirements. There may be mentioned forming agglomerates by extrusion, ringroll - or roll-pressing, die-pressing, rotary table pressing and pelletising, e.g. on a disc pelletiser.

The process may include a self-hardening stage to permit the green briquettes to gain strength, but the briquettes tend to have inadequate water resistance. Preferably, however, a hot curing step is included to speed up the hardening stage and to make the briquettes water resistant, and this may be carried out at temperatures of the order of 200 to 300°C, suitably for about half an hour or more. Hot curing may be conveniently carried out by passing the briquettes on a conveyor through an oven, in an inert or partially inert gas atmosphere which may contain any of nitrogen, carbon dioxide, water vapour and oxygen. It is to be noted that the hot curing step does not correspond to a carbonisation step, and thus not only are there energy savings, but the solid yield on a dry basis is very high. Additionally, there is a reduced risk of pollution.

The release of the green briquettes from the press moulds may be improved, if desired, by prewarming the moulds and/or by sprinkling coal fines or graphite uniformly across the press surface in contact with the mix prior to and during the briquetting of the mix.

The water resistance and appearance of the briquettes may be improved by an additional treatment with a spray or bath of a waterproofing agent. Several agents are known or have been proposed including, for example, aluminium acetate.

The present invention will now be described by way of example only.

### EXAMPLE 1

A fine anthracite, from South Wales, was prepared by drying, crushing and screening to - 3mm. The product was admixed with 8% okf a prepared solution of unrefined molasses sugar (brown sugar) comprising 75% sugar solids and 25% water, and 1% phosphoric acid and 1% iron ore, and the mixture was formed into briquettes using a hydraulic mould-and-plunger press. An initial mean crushing strength of 4.5 kg was measured for the green briquettes.

The briquettes were cured at 250°C for 1½ hours under a mixture of air and nitrogen and after cooling exhibited a mean crushing strength of 87 kg, and an excellent water resistance.

### EXAMPLE 2

The procedure of Example 1 was repeated, but using a commercial starch-derived glucose syrup, containing 80% of sugar solids by weight, comprising dextrose, maltose and higher sugars and 20% water, by weight. Crushing strengths of 3.5 kg and 70 kg were obtained for the green and cured briquettes, respectively, and an excellent water resistance was observed.

### EXAMPLE 3

The procedure of Example 1 was repeated, but using a solution of glucose(dextrose), containing 65% sugar solids and 35% water, by weight and adding 1% phosphoric acid and 2% iron ore. Crushing strengths of 2.5 kg and 80 kg were obtained for the green and cured briquettes, respectively, and an excellent water resistance was observed.

### EXAMPLE 4

The procedure of Example 3 was repeated, but using time at 250°C was reduced to half an hour. After immersion in water for one day, the crushing strength of the briquettes was 126kg.

### EXAMPLE 5

The procedure of Example 1 was repeated, but using a solution of refined sugar (sucrose) containing 65% of sugar solids and 35% of water, by weight, and adding 1% p-toluene sulphuric acid alone. After curing at 250°C for half an hour, followed by immersion in water for one day, the crushing strength of the briquettes was 105kg.

## Claims

1. A cold coal briquetting process characterised by mixing fine coal with a binder comprising 5-15% sugar solution of a concentration of at least 25% by weight and up to 5% of hardening accelerator for the sugar solution selected from iron oxide, calcium carbonate, calcium phosphate and aluminium oxide, each optionally with an acid, and p-toluene sulphonic acid, and forming the mixture into briquettes, and hardening the resulting green briquettes.

2. A process according to claim 1, characterised in that the coal is a high rank non-caking coal.

3. A process according to claim 1 or 2, characterised in that the coal is of particle size below 3mm.

4. A process according to any preceding claim, characterised in that the briquettes are formed by extrusion, ringroll- or roll-pressing, die pressing, rotary table pressing and pelletising.

5. A process according to any preceding claim, characterised in that the hardening includes a hot curing step.

6. A process according to claim 5, characterised in that the briquettes are hardened at 200 - 300°C for at least 0.5 hours.
